

## UNITED STATES PATENT OFFICE

2,092,008

SAPONIFICATION OF CELLULOSE ESTER  
MATERIAL

Robert Wighton Moncrieff, Frank Brentnall Hill,  
and Thomas Barnard Frearson, Spondon, near  
Derby, England, assignors to Celanese Corpora-  
tion of America, a corporation of Delaware

No Drawing. Application December 6, 1934, Se-  
rial No. 756,284. In Great Britain December  
12, 1933

12 Claims.

(Cl. 8—20)

This invention relates to the treatment of cel-  
lulose acetate and other organic esters of cel-  
lulose and particularly to a process for reducing  
the acidyl content of such esters. The invention  
is specially applicable to the saponification of fila-  
ments, threads, yarns, ribbons and the like made  
of or containing such esters.

It has been discovered that organic esters of  
cellulose can be saponified by means of non-  
metallic bases, for example methylamine, ethyl-  
ene diamine and other aliphatic amines, par-  
ticularly those of low molecular weight in the li-  
quid phase, with particular advantage and that  
by treating threads of cellulose acetate and like  
materials in this way specially desirable proper-  
ties may be imparted to the materials. We have  
now found that the saponification of materials  
having a basis of cellulose acetate or other or-  
ganic ester of cellulose by means of non-metallic  
saponifying agents and in particular methyl-  
amine and similar bases may be accelerated to a  
considerable extent by the presence during the  
saponification of heavy metals, i. e. metals other  
than the alkali and alkaline earth metals.

It is to be understood that the term "metal"  
is used in a sense broad enough to include com-  
pounds of the metal. It appears that the metals  
which are most suitable for use in the process of  
the invention are those which are capable of en-  
tering into combination with non-metallic bases,  
for example to form double compounds in which  
the metal is somewhat loosely attached to the  
base, but which show little or no tendency to  
form complex compounds of the metal-amine  
type, such as are formed for example by cobalt,  
chromium and platinum. Among heavy metals  
which are specially suitable for the purpose of  
the invention mention may be made of copper,  
nickel, zinc and silver. The use of copper in  
accelerating the saponifying action of non-metal-  
lic bases is claimed in our co-pending U. S. appli-  
cation S. No. 756,285 filed December 6, 1934.

The metal is preferably added to the saponify-  
ing bath in the form of a soluble salt but may  
also be employed in other forms, for example in  
some cases it is convenient to add the metal in  
the form of an oxide or hydroxide. Preferably  
the metal is added in such a form that it readily  
dissolves in the saponifying bath, and the saponi-  
fying bath may as a result contain a double com-  
pound of the metal with the particular base em-  
ployed. The saponifying bath may contain two  
or more heavy metals capable of accelerating the  
saponification. Other accelerating agents may  
also be present, for example small quantities of

caustic soda or other strong mineral base, as  
claimed in our co-pending U. S. application S.  
No. 756,282, filed December 6, 1934.

The organic ester of cellulose treated may be  
of normal or low viscosity, for example in the case  
of cellulose acetate the viscosity may be of the  
order of 30 to 50, 100, 200 or even higher, these  
figures being obtained by comparison of a 6%  
solution of the ester in acetone at 25° C. with  
glycerine at the same temperature taken as a 10  
standard of 100. Such esters of high viscosity  
may readily be made by methods in which degra-  
dation of the cellulose molecule is substantially  
avoided during acidylation, for example the  
methods of U. S. Patent No. 1,708,787. On the 15  
other hand, the viscosity of the cellulose acetate  
employed may be of the order of 10-20 or even  
lower, or between 20 and 30, measured on the  
scale referred to above.

The invention is of particular importance in 20  
connection with the saponification of filaments,  
threads, ribbons, fabrics and like materials hav-  
ing a basis of cellulose acetate and will be de-  
scribed with special reference to the treatment of  
such materials.

The materials treated may be made by any suit-  
able dry or wet spinning method. Where high  
tenacity is required in the final products it is of  
particular advantage to produce the filaments  
and the like by wet spinning methods in the 30  
course of which they are stretched to a consider-  
able extent, or to soften and stretch the materials  
after their production whether by a wet or a dry  
spinning process. By applying the process of the  
invention to materials which have been stretched 35  
considerably, for example to 200% of their orig-  
inal length or even more, materials of particularly  
valuable serimetric properties are obtainable.

Particularly good results are obtained by the  
use of saponifying baths containing methyl- 40  
amine or ethylene diamine and silver, nickel or  
zinc. Other strong aliphatic organic bases, for  
example ethylamine, propylamine, amyloxine  
and triethylamine, may also be employed. Again,  
somewhat weaker bases of the same se- 45  
ries, for example trimethylamine and allylamine,  
may be used. Further, considerably stronger  
bases of the same series may be employed, even  
very strong bases such as tetramethyl ammonium  
hydroxide, provided care be taken to avoid 50  
damaging the materials. Again, amines other  
than ethylene diamine containing more than  
one amino group, and particularly aliphatic di-  
amines of relatively low molecular weight, for  
example symmetrical dimethyl ethylene diamine, 55

monomethyl ethylene diamine, and propylene diamine may also be used. Preferably at least one of the amino groups of such amines should be unsubstituted or mono-substituted. Amines containing more than two amino groups may also be employed, for example 1,2,3-triaminopropane. The effect of one or more hydroxy groups in the amine appears to be to favour the penetration of the materials by the saponifying agent, and with this object in view substances of the type of  $\alpha\gamma$ -diamino- $\beta$ -hydroxy propane may be used with advantage. Again, bases of the heterocyclic series, for example piperidine may be used.

15 Saponification is preferably effected by subjecting the materials to an aqueous bath containing methylamine or a like acting base and the metal in solution. Generally speaking it is advantageous to employ the base in a concentration of 10-30%, and particularly 15-25%. The temperature of the bath may range from below atmospheric temperature to the neighbourhood of the boiling point of the solution. It is often convenient to work at temperatures between 15 or 20° C. and 25 or 30° C. but when a high degree of saponification is to be effected it is preferable to work at a somewhat higher temperature, e. g. 50-60° C. or 70° C. or even higher, depending on the boiling point of the solution.

25 With a view to preventing excessive evaporation of the base it is of advantage, particularly when working at relatively high temperatures, to cover the surface of the saponifying bath with a layer of an oil, wax or like substance which is immiscible with the bath. The concentrations and temperatures employed in particular cases will naturally depend upon the properties of the particular base employed. In general, the conditions may be chosen so that the desired degree 30 of saponification may be effected by means of a treatment lasting from 1-2 minutes or less up to 3 or 4 minutes. On the other hand the treatment may be more protracted.

35 When the saponifying agent is applied to the materials in the form of an aqueous solution, it is convenient to incorporate the metal, for example in the form of the oxide or hydroxide or of a water-soluble salt, in the saponifying medium itself. It is not, however, essential that the metal should be introduced in this way. It may, for instance, be applied to the materials prior to the application of the saponifying agent, or even introduced into the spinning solution from 40 which they are made.

45 A very considerable acceleration of the saponifying process may be effected by the presence in the saponifying bath of quite small concentrations of the metal, e. g. 0.01-0.05% on the weight of the bath or even less. On the other hand 50 somewhat higher concentrations may be employed, e. g. 0.1% or 0.5%. Since it is undesirable that the final product should contain substantial quantities of the metal it is preferable to work with the smallest quantities capable of giving the desired result.

55 The saponifying medium may also contain swelling agents, solvents or latent solvents for the cellulose ester, for example cyclohexanol, methyl cyclohexanol, glycerol, ethylene glycol and its mono methyl and dimethyl ethers, diacetone alcohol, benzyl alcohol, acetone, dioxane or methylene ethylene ether.

60 When the materials are treated in the form of 75 filaments, threads, yarns and the like, it is of

advantage to effect saponification "in warp formation", i. e. by drawing a large number of ends through the bath in substantially parallel relationship one to another and in the same plane. Thus, yarn may be drawn from a creel by means of rollers or like devices extending across the entire assembly of ends or so-called "warp" and immersed or partially immersed in a bath containing the saponifying agent, through a reed into the bath, and after passing through the bath the materials may be drawn by a second roller, pair of rolls or the like, situated outside the bath, through a reed and out of the bath, whence they are forwarded to suitable collecting means or to means for effecting any subsequent treatment to be applied. Preferably the materials are washed and dried before being wound.

65 The saponifying agent may be applied by other means. Thus, for example, the materials in hank form may be suspended from rods which are caused to traverse the length of the bath, and at the same time to rotate so as to expose each portion of the yarn to the same depth in the bath for the same period. Again, the materials may be treated in the form of bobbins, cheeses or other packages. Any suitable means may in fact be adopted in applying the saponifying agent to the materials. Materials in yarn or like form may be treated continuously with their production and/or with a stretching step. Again, in the case of such materials, stretching may be effected during saponification or, provided saponification has not been carried too far, after saponification. In general it is necessary to soften the materials to enable them to be stretched to the desired extent, and in choosing a suitable softening agent due regard should be had to the extent to which the materials have been saponified.

70 As indicated above, the materials may be saponified in fabric form. This may conveniently be effected by passing the fabric continuously through a bath containing the saponifying agent, for example in an apparatus of the type 45 of the winch dyeing machine.

75 It is generally advisable to treat the materials after saponification so as to remove any metal remaining therein. Any suitable means may be adopted for this purpose. A convenient means comprises washing the materials with a dilute acid with which the particular metal forms a soluble salt.

80 The materials prior to saponification may be subjected to a treatment adapted to facilitate 55 penetration of the saponifying agent. This may comprise the application of water to the materials, or they may be treated with aqueous wetting agents, for example soaps.

85 The degree of saponification effected may be sufficient to reduce the acidyl content of the ester by 8-10% or even less, but is preferably somewhat higher, for example sufficient to reduce the acidyl content by 20-25% or 30%. Considerably higher degrees of saponification may be 60 effected sufficient to remove 35 or 40 to 50 or 55% of the acidyl content or more, even up to complete saponification, according to the particular purpose in view. Generally speaking, a loss in acidyl content of 20-25 or 30% is capable of 70 rendering the cellulose acetate material insoluble in acetone and imparting to it a high affinity for cotton dyes without destroying the affinity for cellulose ester dyes, for example the so-called S. R. A. dyes. The material may be rendered 75

insoluble in substantially anhydrous acetone but may be soluble in acetone containing a considerable percentage, e. g. 25-30%, of water. Or saponification may render the material insoluble in such mixtures as well as in anhydrous acetone. The saponification may raise the safe ironing point considerably. Materials saponified according to the invention may have, in addition to the valuable properties referred to above, a high 10 tenacity and elasticity and a good extensibility. Such materials are of particular value for use in the manufacture of high twist yarns. Thus, high twist yarns partially saponified according to the invention have been found particularly useful as weft in the manufacture of crepe fabrics. Again, by the process of the invention, it is possible to obtain completely saponified materials of excellent tensile properties.

The following examples illustrate the invention:—

*Example 1*

Cellulose acetate yarn is drawn in warp formation through an aqueous bath containing 15-30% of monomethylamine and 0.05-0.05% of silver which is introduced into the bath in the form of silver nitrate. The temperature of the bath is maintained between 50 and 60° C. and the rate of travel of the materials is adjusted so that the 30 yarn is in contact with the bath for 1-3 minutes.

*Example 2*

The process is carried out as described in Example 1 except that the bath comprises a 15-30% aqueous solution of ethylene diamine containing 0.05-0.5% of nickel which is introduced into the bath in the form of nickel sulphate.

Similarly other non-metallic bases, for example propylamine, di-methylamine or others of the bases referred to above may be applied.

Although the invention has been described with particular reference to the treatment of materials having a basis of cellulose acetate, it is also applicable to the treatment of other materials containing other saponifiable esters of cellulose, for example cellulose formate, propionate, butyrate, ethyl cellulose acetate, oxy-ethyl cellulose acetate and nitrocellulose acetate.

What we claim and desire to secure by Letters 50 Patent is:—

1. Process for reducing the acetyl content of an organic ester of cellulose, which comprises saponifying the ester by means of a saponifying agent therefor which is a water-soluble nitrogenous organic base in which each carbon atom that is directly attached to a nitrogen atom is directly attached to three other atoms apart from said nitrogen atom, in the presence in solution of metal selected from the group consisting of 55 nickel, zinc, and silver.

2. Process for saponifying filaments, threads, ribbons and like materials having a basis of organic ester of cellulose, which comprises treating the materials with an aqueous solution of a 60 saponifying agent therefor which is a water-soluble nitrogenous organic base in which each carbon atom that is directly attached to a nitrogen atom is directly attached to three other atoms apart from said nitrogen atom, in the presence in 65 solution of a metal selected from the group consisting of nickel, zinc and silver.

3. Process for saponifying filaments, threads, ribbons and like materials having a basis of cellulose acetate, which comprises treating the materials with an aqueous solution of a saponifying 70

agent therefor which is a water-soluble nitrogenous organic base in which each carbon atom that is directly attached to a nitrogen atom is directly attached to three other atoms apart from said nitrogen atom, in the presence in solution of 5 metal selected from the group consisting of nickel, zinc and silver.

4. Process for saponifying filaments, threads, ribbons and like materials having a basis of cellulose acetate, which comprises treating the materials with an aqueous bath containing a water-soluble nitrogenous organic base in which each carbon atom that is directly attached to a nitrogen atom is directly attached to three other atoms apart from said nitrogen atom which is a 10 saponifying agent for the organic ester of cellulose and a double compound of said base with a metal selected from the group consisting of nickel, zinc and silver.

5. Process for saponifying filaments, threads, 20 ribbons and like materials having a basis of organic ester of cellulose, which comprises treating the materials with an aqueous solution of a saponifying agent therefor which is a water-soluble nitrogenous organic base in which each carbon 25 atom that is directly attached to a nitrogen atom is directly attached to three other atoms apart from said nitrogen atom, in the presence of nickel in solution.

6. Process for saponifying filaments, threads, 30 ribbons and like materials having a basis of organic ester of cellulose, which comprises treating the materials with an aqueous solution of a saponifying agent therefor which is a water-soluble nitrogenous organic base in which each 35 carbon atom that is directly attached to a nitrogen atom is directly attached to three other atoms apart from said nitrogen atom, in the presence of zinc in solution.

7. Process for saponifying filaments, threads, 40 ribbons and like materials having a basis of organic ester of cellulose, which comprises treating the materials with an aqueous solution of a saponifying agent therefor which is a water-soluble nitrogenous organic base in which each carbon 45 atom that is directly attached to a nitrogen atom is directly attached to three other atoms apart from said nitrogen atom, in the presence of silver in solution.

8. Process for saponifying filaments, threads, 50 ribbons and like materials having a basis of cellulose acetate, which comprises treating the materials with an aqueous solution of an amine selected from the group consisting of mono-methylamine, mono-ethylamine and ethylene diamine, in the presence of nickel in solution.

9. Process for saponifying filaments, threads, 55 ribbons and like materials having a basis of cellulose acetate, which comprises treating the materials with an aqueous solution of an amine selected from the group consisting of mono-methylamine, mono-ethylamine and ethylene diamine, in the presence of zinc in solution.

10. Process for saponifying filaments, threads, 60 ribbons and like materials having a basis of cellulose acetate, which comprises treating the materials with an aqueous solution of an amine selected from the group consisting of mono-methylamine, mono-ethylamine and ethylene diamine, in the presence of silver in solution.

11. Process for saponifying filaments, threads, 70 ribbons and like materials having a basis of organic ester of cellulose, which comprises treating the materials with an aqueous medium containing in solution an amine of relatively low molecu- 75

lar weight which is a saponifying agent for the organic ester of cellulose and a metal selected from the group consisting of nickel, zinc and silver.

5 12. Process for saponifying filaments, threads, ribbons and like materials having a basis of cellulose acetate, which comprises treating the materials with an aqueous medium containing in

solution an amine of relatively low molecular weight which is a saponifying agent for cellulose acetate and a metal selected from the group consisting of nickel, zinc and silver.

ROBERT WIGHTON MONCRIEFF.  
FRANK BRENTNALL HILL.  
THOMAS BARNARD FREARSON.